# EUROPEAN PATENT SPECIFICATION

(11) **EP 1 481 712 B1**
(45) Date of publication and mention of the grant of the patent: **10.05.2006**
(21) Application number: 03012021.6
(22) Date of filing: 28.05.2003
(51) Int. Cl.: A63C 5/12

(54) **Running surface for a winter sports apparatus, winter sports apparatus comprising such running surface, material composition for production of such running surface, use of a material additive to such running surface and method of manufacture of such running surface**
Laufsohle für ein Wintersportgerät, Wintersportgerät mit solch einer Laufsohle, Materialzusammensetzung für die Herstellung solch einer Laufsohle, Verwendung eines Materialzusatzes für solch eine Laufsohle und Verfahren zur Herstellung solch einer Laufsohle
Semelle de glisse pour appareil de sport d'hiver, appareil de sport d'hiver utilisant une telle semelle de glisse, composition pour une telle semelle de glisse, usage d'additif pour une telle semelle de glisse et méthode de production d'une telle semelle de glisse

(43) Date of publication of application: 01.12.2004
(73) Proprietor: IMS KUNSTSTOFF AG, 3076 Worb (CH)
(72) Inventor: Geissbühler, Urs, 3604 Thun (CH); Cebocli, Aude, 73490 La Ravoire (FR); Garcin, Pierre, 73410 Saint Ours (FR)
(74) Representative: Hepp, Dieter

(56) References cited:
- CH-A- 657 993
- FR-A- 2 719 050

## Description

The invention relates to a running surface for a winter sports apparatus, more precisely to the enhancement of the gliding properties of such a running surface.

Currently used running surfaces for winter sports apparatus, e.g. any types of skis (e.g. cross-country skis, alpine skis, telemark skis), snowboards, skiboards, sleds etc., in more general terms for any running surface intended for gliding on snow or ice are preferably made of hydrophobic plastics, e.g. polyethylene (PE). The mechanism of gliding of such running surfaces on snow and/or ice is yet not fully understood. However, it is believed that upon interaction of surface roughness and snow- or ice crystals a hydrodynamic lubricating effect upon melt water due to frictional heat is essentially involved.

At higher gliding speed, the locally formed melt water tends to spread all over the running surface, leading to an unwanted "suction effect" which may influence the gliding speed in a negative way. In order to overcome this phenomenon, additives such as soot, carbon black and graphite have been added to the polyethylene matrix (see e.g. CH 657 993 A and CH 660 018 A). These additives are supposed to diminish the "suction effect" due to their higher heat conductivity. The superior gliding properties of such modified running surfaces led to their preferential use today. However, these running surfaces are inevitably black due to the black color of soot, carbon black and graphite, thus hampering any alternative coloration of running surfaces. Moreover, there is a high need for further improved gliding properties of running surfaces, especially for sports competition purposes.

It is an object of the present invention to avoid the shortcomings of the known running surfaces and particularly to provide a running surface for winter sports apparatus with further improved gliding properties. It is an additional object of the invention, to provide a running surface for winter sports apparatus that allow for a non-black coloration. Such running surfaces need to be inexpensively and easy to produce and to apply. Moreover, the running surfaces have to meet the demands of high durability.

The above-mentioned objects are fulfilled by a running surface for a winter sports apparatus, a winter sports apparatus comprising such a running surface, a material composition for the production of such running surface and a method of manufacture such running surfaces according to the independent claims.

The invention concerns a running surface for a winter sports apparatus or the like, e.g. any types of skis (e.g. cross-country skis, alpine skis, telemark skis), snowboards, skiboards, sleds etc., in more general terms any types of running surfaces intended for gliding on snow or ice wherein the running surface contains a mineral addition chosen from the sodalite group and tsaregorodtsevite-wadalite series or a mixture thereof. Explicitly enclosed within the intention of the invention are also naturally and non-naturally occuring closely related structural and/or chemical analogues of these minerals, especially the derivatives obtainable by exchange of the cation(s) or anion(s). The nomenclature of these mineral additions is given according to the Strunz Classification System [Hugo Strunz; Ernest Nickel: Strunz Mineralogical Tables. Ninth Edition. 2001. ISBN 3-510-65188-X], where the sodalite group and tsaregorodtsevite-wadalite series is classified under VIII/J.11 (Tectosilicates). Typical members of this class are:
Tsaregorodtsevite, VIII/J.11-05, N(CH₃)₄[Si₂(Si_{0.5}Al_{0.5})O₆]₂;
Sodalite, VIII/J.11-10, Na₄Al₃Si₃O₁₂Cl;
Nosean, VIII/J. 11-20, Na₈Al₆Si₆O₂₄(SO₄);
Hauyne, VIII/J. 11-30, (Na,Ca)₄₋₈[Al₆Si₆(O,S)₂₄](SO₄,Cl)₁₋₂;
Lazurite, VIII/J. 11-40, (Na,Ca)₈(AlSiO₄)₆(S,SO₄,Cl)₁₋₂;
Tugtupite, VIII/J.11-50, Na₄AlBeSi₄O₁₂Cl;
Kamaishilite, VIII/J.11-60, Ca₂Al₂SiO₆(OH)₂; and
Bicchulite, VIII/J.11-70, Ca₂Al₂SiO₆(OH)₂.

It has now surprisingly been found that such a mineral addition further improves the gliding properties of running surfaces to a remarkable extent. In order to improve the gliding properties of running surfaces, soot, carbon black or graphite can be substituted with these mineral additions. Moreover, due to the color of these minerals, a non-black coloration of running surfaces is easily achievable. The running surfaces according to the invention are inexpensively and easy to produce, are easy to apply and fulfill the demands of durability. Of course, the running surface according to the invention may be used with or without a layer of wax for the purpose of gliding enhancement.

In a preferred embodiment, a running surface according to the invention is made of plastic, especially of polyethylene (PE). Preferentially, ultra high molecular weight (UHMW) polyethylene (PE) e.g. in the range of about 2 x 10⁶ g/mol to about 12 x 10⁶ g/mol of high density is used for this purpose and processed in a press-sintering process. However, the running surface according to the invention may also be produced by extrusion of high density polyethylene (PE) with a molecular weight in the range of about 2 x 10⁵ g/mol to 8 x 10⁵ g/mol. Of course, the invention is not limited to the use of a specific polymer matrix and can be carried out with any other preferably hydrophobic plastic material as well, that are useful for the production of such running surfaces.

In an especially preferred embodiment, the mineral addition contains an ultramarine; optionally, further especially mineral additions may be included in the running surface. Ultramarines such as the naturally occuring lazurite (Strunz ID: VIII/J.11-40, the blue component of the gemstone lapis lazuli) are also known under the synonyms cyaneus, lasurite (of Brogger), Lasurstein, lazurite (of Dana), Sapphis (of Agricola). Beside their natural occurence, ultramarines of the general formula Na₄[Al₃Si₃O₁₂]S₃ can be synthesized by fusing kaolin, sodium carbonate and sulfur, rendering them particularly useful for large-scale purposes for cost reasons. With ultramarines, especially advantageous gliding properties are obtainable, in some embodiments even exceeding the effect of soot, carbon black and graphite at comparable or less amounts to be added. Moreover, due to the strong coloration effect of ultramarines, new colorations of running surfaces are obtainable without a negative effect to the gliding properties. Besides a blue coloration (e.g. due to ultramarineblue, C.A.S. no. 57455-37-5), especially pink or violet (C.A.S. no. 12769-96-9) variations of ultramarines are of course also to be used in accordance with the invention in order to achieve more different colorations.

Most preferably, the mineral addition contains about 0.1% to about 40% by weight, preferably about 1% to about 30% by weight of an ultramarine. This range proved especially effective in enhancing the gliding properties without significantly altering stability, flexibility or other mechanical and/or physical properties of the running surface.

In accordance with yet another preferred embodiment of the invention, the running surface additionally contains soot and/or carbon black and/or graphite. Experimental results indicate that both these classes of additives can be synergistically incorporated into a running surface simultaneously, providing an especially advantageous influence on the gliding characteristic of the running surface.

According to an especially preferred embodiment of the invention, the running surface comprises about 75% to about 95% by weight, preferably about 85% by weight of polyethylene, 0% to about 20% by weight, preferably about 10% by weight of soot and/or carbon black and/or graphite and about 0.1% to about 40% by weight, preferably about 1% to about 30% by weight, most preferably about 5% by weight of a mineral addition chosen from the sodalite group and tsaregorodtsevite-wadalite series or a closely related structural and/or chemical analogue thereof, preferably an ultramarine. Compositions comprising these amounts of additives proved especially advantageous with respect to gliding properties, mechanical and handling properties and coloration.

A material composition for the production of a running surface comprises preferably polyethylene and a mineral addition chosen from the sodalite group and tsaregorodtsevite-wadalite series or a closely related structural and/or chemical analogue thereof, preferably an ultramarine. Optionally, soot, carbon black or graphite may be included. A material composition is here and henceforth to be understood including the still unprocessed mixture of crude materials as well as especially a press-sintered body produced from such mixture, from which a running surface can be peeled down.

Obviously, the use of a mineral chosen from the sodalite group and tsaregorodtsevite-wadalite series or a mixture thereof, especially an ultramarine as additive to a running surface of a winter sports apparatus is especially advantageous.

A running surface according to the invention can be produced in a sintering or extrusion process, comprising the step of adding a mineral addition chosen from the sodalite group and tsaregorodtsevite-wadalite series or a mixture thereof, especially an ultramarine.

The invention will now be exemplarily described by means of preferred embodiments; however, the invention is not to be limited to these embodiments.

### Example 1 (for comparative purposes, state of the art)

A mixture of 15 parts by weight of carbon black (20nm particle size; oil necessity of 500%) and 85 parts by weight of the high density polyethylene Hostalen GUR 4170 (molecular weight 10,5 x 10⁶ g/mol) is prepared in a mixing apparatus. The mixture is then press-sintered to a homogeneous cylindrical body according to standard procedures (e.g. such as those disclosed in the brochure of Hoechst, "Hostalen GUR" [HKR112-7089C12299/14]). After cooling down, the cylindrical body is peeled down to a band with the thickness of a running surface, e.g. 1,4 mm. The running surface is then roughened on one side and prepared for fixation on the ski body with an oxidizing flame. Of course, the running surface may also be prepared by an extrusion process. The general process of production is not essential to the invention, but rather the nature of the additive(s) to the running surface.

### Example 2 (according to the invention)

Example 1 is repeated, but the composition of the starting mixture is altered to 100 parts by weight of the polyethylene component and 1 part by weight of ultramarine (C.A.S. no. 57455-37-5).

### Example 3 (according to the invention)

Example 1 is repeated, but the composition of the starting mixture is altered to 85 parts by weight of the polyethylene component, 10 parts by weight of the carbon black component and 5 parts by weight of ultramarine (C.A.S. no. 57455-37-5).

### Example 4 (according to the invention)

Example 1 is repeated, but the composition of the starting mixture is altered to 76 parts by weight of the polyethylene component, 4 parts by weight of the carbon black component and 20 parts by weight of ultramarine (C.A.S. no. 57455-37-5).

### Measurements, physical properties

Running surfaces according to examples 1 to 4 were characterized by means of some of their physical characteristics (table 1). No outstanding differences were detected that might significantly contribute to a change of gliding properties.

**Table 1: physical characteristics of running surfaces according to examples 1 to 4.**

| | Example 1 | Example 2 | Example 3 | Example 4 |
|---|---|---|---|---|
| density [g/cm³] | 1.002 | 0.948 | 1.011 | 1.062 |
| min. melting point [°C] | 139.7 | 141.0 | 139.3 | 140.0 |
| melting enthalpy [J/g] | 129 | 140 | 129 | 92 |

### Gliding properties

Skis were prepared comprising running surfaces according to examples 1 to 4. For the gliding test purpose, skis were used that are built around a central core, comprising a supporting laminate structure on the top and bottom of the core, the gliding surface being fixed between lateral running edges. However, the running surface according to the invention may of course be used with any type of winter sports apparatus intended for gliding on snow or ice. Beside the different running surfaces, the skis were constructed equivalently. Skis comprising running surfaces according to the invention (examples 2 to 4) exhibited comparable or improved gliding properties in comparison to the ski comprising a running surface according to the prior art (example 1).

## Claims

1. Running surface for a winter sports apparatus, **characterised in that** the running surface contains a mineral addition chosen from the sodalite group and tsaregorodtsevite-wadalite series or a mixture thereof.

2. Running surface according to claim 1, **characterised in that** the running surface is made of plastic, especially of polyethylene (PE).

3. Running surface according to claims 1 or 2, **characterised in that** the mineral addition contains an ultramarine.

4. Running surface according to one of claims 1 to 3, **characterised in that** the mineral addition contains about 0.1% to about 40% by weight, preferably about 1% to about 30% by weight of an ultramarine.

5. Running surface according to one of claims 1 to 4, **characterised in that** the running surface additionally contains soot and/or carbon black and/or graphite.

6. Running surface according to claim 5, **characterised in that** the running surface comprises about 75% to about 95% by weight, preferably about 85% by weight of polyethylene, 0% to about 20% by weight, preferably about 10% by weight of soot and/or carbon black and/or graphite and about 0.1% to about 40% by weight, preferably about 1% to about 30% by weight, most preferably about 5% by weight of a mineral addition chosen from the sodalite group and tsaregorodtsevite-wadalite series or a closely related structural and/or chemical analogue thereof, preferably an ultramarine.

7. Winter sports apparatus, comprising a running surface according to one of claims 1 to 6.

8. Material composition for the production of a running surface according to one of claims 1 to 6, **characterised in that** it comprises polyethylene and a mineral addition chosen from the sodalite group and tsaregorodtsevite-wadalite series or a closely related structural and/or chemical analogue thereof, preferably an ultramarine.

9. Use of a mineral chosen from the sodalite group and tsaregorodtsevite-wadalite series or a mixture thereof, especially an ultramarine as additive to a running surface of a winter sports apparatus.

10. Method of manufacture of a running surface for a winter sports apparatus in a sintering or extrusion process, comprising the step of adding a mineral addition chosen from the sodalite group and tsaregorodtsevite-wadalite series or a mixture thereof, especially an ultramarine.

## Patentansprüche

1. Laufsohle für ein Wintersportgerät, **dadurch gekennzeichnet, daß** die Laufsohle einen Mineralzusatz enthält, der aus der Sodalithgruppe und der Tsaregorodtsevit-Wadalit-Reihe oder einem Gemisch davon ausgewählt ist.

2. Laufsohle nach Anspruch 1, **dadurch gekennzeichnet, daß** die Laufsohle aus Kunststoff, insbesondere aus Polyethylen (PE), hergestellt ist.

3. Laufsohle nach Anspruch 1 oder 2, **dadurch gekennzeichnet, daß** der Mineralzusatz ein Ultramarin enthält.

4. Laufsohle nach einem der Ansprüche 1 bis 3, **dadurch gekennzeichnet, daß** der Mineralzusatz etwa 0,1 Gew.% bis etwa 40 Gew.%, vorzugsweise etwa 1 Gew.% bis etwa 30 Gew.%, eines Ultramarins enthält.

5. Laufsohle nach einem der Ansprüche 1 bis 4, **dadurch gekennzeichnet, daß** die Laufsohle außerdem Ruß und/oder Rußschwarz und/oder Graphit enthält.

6. Laufsohle nach Anspruch 5, **dadurch gekennzeichnet, daß** die Laufsohle etwa 75 Gew.% bis etwa 95 Gew.%, vorzugsweise etwa 85 Gew.%, Polyethylen, 0 Gew.% bis etwa 20 Gew.%, vorzugsweise etwa 10 Gew.%, Ruß und/oder Rußschwarz und/oder Graphit und etwa 0,1 Gew.% bis etwa 40 Gew.%, vorzugsweise etwa 1 Gew.% bis etwa 30 Gew.%, am stärksten bevorzugt etwa 5 Gew.%, eines Mineralzusatzes, ausgewählt aus der Sodalithgruppe und der Tsaregorodtsevit-Wadalit-Reihe oder einem nahe verwandten strukturellen und/oder chemischen Analogen davon, vorzugsweise ein Ultramarin, umfaßt.

7. Wintersportgerät, das eine Laufsohle nach einem der Ansprüche 1 bis 6 aufweist.

8. Materialzusammensetzung für die Herstellung einer Laufsohle nach einem der Ansprüche 1 bis 6, **dadurch gekennzeichnet, daß** sie Polyethylen und einen Mineralzusatz, ausgewählt aus der Sodalithgruppe und der Tsaregorodtsevit-Wadalit-Reihe oder einem nahe verwandten strukturellen und/oder chemischen Analogen davon, vorzugsweise ein Ultramarin, umfaßt.

9. Verwendung eines Minerals, ausgewählt aus der Sodalithgruppe und der Tsaregorodtsevit-Wadalit-Reihe oder einem Gemisch davon, insbesondere eines Ultramarins, als Zusatzstoff zu einer Laufsohle eines Wintersportgeräts.

10. Verfahren zur Herstellung einer Laufsohle für ein Wintersportgerät in einem Sinter- oder Extrusionsverfahren, das den Schritt des Zusetzens eines Mineralzusatzes, ausgewählt aus der Sodalithgruppe und der Tsaregorodtsevit-Wadalit-Reihe oder einem Gemisch davon, insbesondere ein Ultramarin, umfaßt.

## Revendications

1. Semelle de glisse pour un appareil de sports d'hiver, **caractérisée en ce qu'**elle contient un additif minéral choisi parmi le groupe de la sodalite, la série de la tsaregorodtsevite-wadalite, ou un mélange de ceux-ci.

2. Semelle de glisse selon la revendication 1, **caractérisée en ce qu'**elle est constituée d'une matière plastique, en particulier de polyéthylène (PE).

3. Semelle de glisse selon la revendication 1 ou 2, **caractérisée en ce que** l'additif minéral contient un outremer.

4. Semelle de glisse selon l'une des revendications 1 à 3, **caractérisée en ce que** l'additif minéral contient environ 0,1 % à environ 40 % en poids, de préférence environ 1 % à environ 30 % en poids, d'un outremer.

5. Semelle de glisse selon l'une des revendications 1 à 4, **caractérisée en ce qu'**elle contient en outre de la suie et/ou du noir de carbone et/ou du graphite.

6. Semelle de glisse selon la revendication 5, **caractérisée en ce qu'**elle comprend environ 75 % à environ 95 % en poids, de préférence environ 85 % en poids de polyéthylène, 0 % à environ 20 % en poids, de préférence environ 10 % en poids de suie et/ou de noir de carbone et/ou de graphite, et environ 0,1 % à environ 40 % en poids, de préférence environ 1 % à environ 30 % en poids, de la manière la plus préférée environ 5 % en poids, d'un additif minéral choisi parmi le groupe de la sodalite, la série de la tsaregorodtsevite-wadalite, ou un analogue structurel et/ou chimique étroitement apparenté à ceux-ci, de préférence un outremer.

7. Appareil de sports d'hiver, comprenant une semelle de glisse selon l'une des revendications 1 à 6.

8. Composition de matériau pour la production d'une semelle de glisse selon l'une des revendications 1 à 6, **caractérisée en ce qu'**elle comprend un polyéthylène et un additif minéral choisi parmi le groupe de la sodalite, la série de la tsaregorodtsevite-wadalite, ou un analogue structurel et/ou chimique étroitement apparenté à ceux-ci, de préférence un outremer.

9. Utilisation d'un minéral choisi parmi le groupe de la sodalite, la série de la tsaregorodtsevite-wadalite ou un mélange de ceux-ci, en particulier un outremer, en tant qu'additif pour une semelle de glisse d'un appareil de sports d'hiver.

10. Procédé pour fabriquer une semelle de glisse pour un appareil de sports d'hiver, dans un processus de frittage ou d'extrusion, comprenant l'étape consistant à ajouter un additif minéral choisi parmi le groupe de la sodalite, la série de la tsaregorodtsevite-wadalite, et un mélange de ceux-ci, en particulier un outremer.
